

## UNITED STATES PATENT OFFICE

HENRY L. COLES, OF HAMILTON, OHIO, ASSIGNOR TO GUARDIAN METALS COMPANY, OF HAMILTON, OHIO, A CORPORATION OF DELAWARE

## FERROUS ALLOYS

No Drawing.

Application filed March 22, 1930. Serial No. 438,232.

This invention relates to improvements in ferrous alloys, and more particularly to an improved composition comprising manganese, chromium and carbon in substantial amounts.

5 Hitherto metals requiring a high degree of hardness and torch resistance, have included major proportions of tungsten and its compounds as well as analogous metals and their compounds, together with substantial amounts of carbon, in alloy form. Such materials, while efficient, are costly to manufacture and require special precautions in the preparation of the various alloys thereof and in the fabrication of articles prepared therefrom.

10 It is an object of the present invention to provide an improved ferrous alloy having a high degree of hardness and torch resistance.

15 It is also an object of this invention to provide an improved ferrous alloy containing substantial amounts of manganese, chromium and carbon.

20 Another object of this invention is to provide an improved composition comprising major amounts of iron and substantial amounts of combined manganese, chromium, and carbon.

25 These, and other desirable objects and advantages of the present invention will be described in the accompanying specification, certain preferred compositions being disclosed by way of example only, for, since the improvements of the present invention may be comprehended in other specific compositions, it is not intended to be herein limited to the ones set forth as examples except as such limitations are clearly imposed by the appended claims.

30 In one of the desired practical embodiments the improved alloy of the present invention preferably comprises substantially 15 to 18 per cent manganese, 7 to 15 per cent chromium, 2.2 to 3 per cent carbon, and the remainder iron. While these percentages have been set forth as determinative of the preferred range of the compositions included in this invention, it will, of course, be understood that variations in the amounts of the several components may be made without de-

parting from the spirit and scope of this invention. As exemplifying specific compositions which have been found to give desirable results, the following are noted:

| No. | % Mn  | % Cr  | % C  | % Fe  | 55 |
|-----|-------|-------|------|-------|----|
| 1   | 16.51 | 9.03  | 2.19 | 72.37 |    |
| 2   | 14.17 | 10.72 | 2.75 | 72.36 |    |
| 3   | 17.14 | 15.47 | 2.53 | 64.86 |    |
| 4   | 18.00 | 7.45  | 2.76 | 71.79 | 60 |

60 All of the alloys above described have a scratch hardness of substantially 7.4 to 9 on Moh's scale, and are markedly torch-resistant and drill resistant.

65 While a preferred range of compositions has been disclosed, the invention comprehends alloys included within varying percentages, as follows:

|           |                   |    |
|-----------|-------------------|----|
| Manganese | 13 to 20 per cent | 65 |
| Chromium  | 3 to 18 per cent  | 70 |
| Carbon    | 2 to 4 per cent   |    |
| Iron      | 82 to 61 per cent |    |

75 In the preparation of improved alloys of the present invention, the material is melted in any desirable type of furnace but preferably in an indirect arc electric furnace. Typical furnace charges may be recited as follows:

|                |                   |    |
|----------------|-------------------|----|
| Spiegel pig    | 81 to 86 per cent | 70 |
| Ferromanganese | 3 to 2 per cent   |    |
| Ferrochromium  | 16 to 12 per cent |    |

76 When using scrap from the castings made from the above, the following preparations were found to be satisfactory:

|                |                   |    |
|----------------|-------------------|----|
| Spiegel pig    | 46 to 57 per cent | 75 |
| Ferromanganese | 1 to 2 per cent   |    |
| Ferrochromium  | 6 to 11 per cent  |    |
| Alloy scrap    | 47 to 30 per cent | 90 |

80 The analysis for manganese, chromium and carbon in the raw materials used is as follows:

|                |                          |    |
|----------------|--------------------------|----|
| Ferromanganese | 8.4 per cent manganese   | 85 |
|                | 4.65 per cent carbon     |    |
| Ferrochromium  | 80.3 per cent chromium   |    |
|                | 1.49 per cent carbon     |    |
| Spiegeleisen   | 20.11 per cent manganese |    |
|                | 2.97 per cent carbon     |    |

90 It is preferred to employ the rocking in-

direct-arc electric furnace in the preparation of these improved alloys. One desired purpose for using this type of furnace is to substantially eliminate the burning out of manganese from the composition as well as to insure homogeneity of the resulting product.

The metal, after melting, is preferably allowed to set in the ladles until it becomes substantially quiet. It is then poured into molds which are preferably pre-heated. This pouring is usually done rapidly and the castings are allowed to cool slowly for a desired period to prevent cracking. This cooling may even extend for twenty-four hours. One method of accomplishing the desired cooling is to ram up the molds with an excess thickness of sand to thereby retard the dissipation of heat from the casting. Such regulated cooling acts to equalize the stresses normally set up in the casting.

It will now be appreciated that there has been described novel ferrous alloy compositions having relatively high manganese and chromium contents, together with a high carbon content, and which are characterized by a very marked degree of torch and drill resistance.

It will be particularly noted from the foregoing description that the improved alloy described herein accomplishes in a much more efficient manner the heat resistance and drill resistance desired. Further, these advantages are obtained by an alloy which is very much reduced in cost of manufacture, and gives many advantages not obtained in some of the other alloys. This improved alloy is capable of many uses, especially where it is desired to employ material which will readily withstand heat and is especially resistant to the action of drills and other destructive implements.

The improved alloy herein set forth and described is defined as an example, and it is desired that any modifications or changes therein shall be considered as being within the scope of this invention as outlined in the following claims.

What is claimed is:

- 50 1. A hard alloy comprising 14 to about 18% manganese, 7 to 9.03% chromium, about 2 to 4% carbon and the balance iron.
2. A hard alloy comprising about 16.5% manganese, about 9.03% chromium, about 55 2.19% carbon and the balance iron.
3. A hard alloy comprising about 18% manganese, about 7.45% chromium, about 2.76% carbon, and the balance iron.
4. A hard alloy comprising about 16 to 60 18% manganese, about 8 to less than 9% chromium, and about 2 to 3.5% carbon and the balance iron.

This specification signed this 21 day of March, 1930.